

1

3,149,906  
PROCESS FOR TREATING ANIMAL FIBERS  
WITH OZONE

Walter J. Thersen, El Cerrito, Calif., assignor to the  
United States of America as represented by the Secretary  
of Agriculture  
No Drawing. Filed Mar. 11, 1963, Ser. No. 265,583  
3 Claims. (Cl. 8—128)  
(Granted under Title 35, U.S. Code (1952), sec. 266)

A non-exclusive, irrevocable, royalty-free license in  
the invention herein described, throughout the world for  
all purposes of the United States Government, with the  
power to grant sublicenses for such purposes, is hereby  
granted to the Government of the United States of America.

This invention relates to and has among its objects  
the provision of novel processes for treating animal  
fibers, particularly wool, mohair, and the like, with ozone  
in order to improve their properties. Further objects of  
the invention will be evident from the following description  
wherein parts and percentages are by weight unless  
otherwise specified.

As a general proposition, the treatment of wool with  
ozone has been described heretofore and has been sug-  
gested as a means of improving the shrinkage properties  
of the textile and increasing its affinity for dyes. Various  
investigators have explored the situation and have advo-  
cated different techniques for accomplishing their de-  
sired ends. A typical procedure is that described in  
British Patent No. 242,027, November 5, 1925. In this  
process, wool is soaked in 5% ammonia solution for a  
few minutes, hydro-extracted (centrifuged) to remove  
excess liquid, then placed while damp in a chamber  
wherein it is exposed to air containing ozone in a concen-  
tration of about 1 part per 1000. The process is ex-  
ceedingly slow as evidenced by the fact that the patentees  
suggest removing samples of the wool "at intervals of  
a few hours" to test them for acidity. (If acid, the wool  
is again soaked in ammonia solution prior to further  
ozone treatment.) The procedure of the British patent,  
termed the "Zair" process, was further investigated by  
Brown (Journal of the Society of Dyers and Colourists,  
vol. 44, pp. 230-233, 1928), who illustrates the long  
duration of the procedure, i.e. 5 to 20 hours, and sug-  
gests that maximum increase in dye absorption proper-  
ties is attained when the wool is treated with ozone for  
15 hours. In addition to requiring long processing times,  
the various prior procedures have involved such disad-  
vantages as erratic and non-uniform results, decrease in  
abrasion resistance of the treated wool, and even loss of  
material during processing by dissolving of a portion of  
the fibers. As a net result the ozone treatment of wool  
has not met with commercial acceptance.

The process of the invention surmounts the difficulties  
above and leads to the following particular advantages:

A primary item is that the process of the invention  
requires a brief period of time, that is, usually about 3 to  
6 minutes and at most about 10 minutes. Despite this  
short processing time, the treated fibers display many  
improvements in their properties, namely:

The resistance of the fibers to felting and shrinking  
is markedly improved.

The treated fibers are whiter than the original (un-  
treated) fibers.

The treated fibers take up dyes more rapidly than the  
untreated fibers. In addition, the fastness of the dyes to  
the ozone-treated wool is unchanged and fading resistance  
is equal to or better than with the dyed untreated wool.

2

The treated product displays increased fiber cohesive  
forces; that is, the individual fibers cling to one another  
more tenaciously than is the case with the untreated  
material. This in turn provides these benefits: Yarns  
can be spun to a higher count, that is, to finer diameter  
or fewer fibers per cross-section. Yarns can be fabri-  
cated with less twist than from the untreated fibers, yet  
without any loss in yarn tensile strength. (Yarns with  
less twist are especially desirable for fabricating gar-  
ments as the products have improved wrinkle recovery).  
Finer yarns can be spun from the treated fibers and with  
greater efficiency, e.g., with fewer breaks.

In addition to these advantages noted above, the treat-  
ment in accordance with the invention does not produce  
any degradative effect so that there is no detriment in  
what may be termed the purely mechanical properties of  
the material. Thus, there is no loss in tensile strength or  
abrasion resistance. In addition, the material retains its  
original hand so that it is suitable for fabrication of  
garments of all kinds such as suits, skirts, shirts, etc.

In essence, the process of the invention involves con-  
tacting the fibrous material with a current of steam and  
ozone. Various conventional types of textile-treating de-  
vices can be adapted for achieving the desired contact  
between the material and the steam-ozone mixture. Typi-  
cally, for batch operations one may provide a chamber  
supplied with perforated shelves, a gas inlet, an exhaust  
vent, and a discharge outlet for condensed water. The  
fibrous material to be treated is laid on these shelves  
and a stream of the steam-ozone mixture is directed into  
the chamber, preferably in such a manner that it actually  
passes through the material, or, more accurately, through  
the interstices between individual fibrous elements. For  
continuous treatment of long lengths of material such  
as yarns, slivers, top, cloth, etc., the material can be  
threaded over a series of perforated rollers supplied  
through hollow shafts, with the steam-ozone mixture  
which then flows through the material as it passes over  
each roller.

Generally, the ozone is produced in a conventional de-  
vice wherein oxygen is passed through an electrical sys-  
tem involving a high-voltage silent discharge. The efflu-  
ent gas from this device contains, for example, about from  
10 to 100 mg. of ozone per liter, depending on the cir-  
cuit adjustments of the device. (The portion of this  
gas stream which is not ozone is, of course, oxygen.)  
This gas stream is mixed with a stream of steam pro-  
duced by a conventional steam generator. The relative  
proportions of steam and ozone are so adjusted that the  
steam-ozone mixture has an ozone concentration of about  
10 to 50 mg. per liter. The temperature at which the  
process of the invention is carried out may be varied from  
about 60 to 95° C. Temperature control of the treat-  
ment is most readily achieved by adjustment of the tem-  
perature of the steam-ozone stream. This in turn is  
readily controlled by adjustment of the proportions of  
steam and ozone which are combined. For example,  
by increasing the proportion of steam in relation to the  
proportion of ozone coming from the ozone generator,  
the temperature of the steam-ozone composite stream  
may be increased.

The time of contact between the fibrous material and  
the steam-ozone mixture may be varied depending on  
such conditions as the reaction temperature, the concen-  
tration of ozone in the steam-ozone mixture, the type  
of fibrous material being treated, and the degree of modi-  
fication of the fibrous material which is desired. For  
example, an increase in reaction temperature or an in-

The results obtained are summarized below:

| Run | Temperature of treatment, °C. | Ozone concentration in steam-ozone mixture, mg./liter | Area shrinkage,* percent |
|-----|-------------------------------|-------------------------------------------------------|--------------------------|
| 10  | 87                            | 19.6                                                  | 4.0                      |
|     | 83                            | 22.0                                                  | 6.0                      |
|     | 79                            | 27.7                                                  | 4.0                      |
|     | 75                            | 31.4                                                  | 0                        |

\*Shrinkage of untreated wool was 42%.

*Example II*

crease in ozone concentration will increase the speed of modification. In any particular case, pilot trials may be conducted with the material to be treated, employing various conditions and testing the properties of the product. From such tests the appropriate conditions may be easily derived. In such trials, the shrinkage characteristics of the product may, for example, be used as the criterion and the conditions of reaction selected so that the area shrinkage of the product (tested by a standard method) is markedly improved, i.e. reduced to at least one-half, preferably at least one-tenth, of that displayed by the starting (untreated) material. It is, of course, obvious that the process should not be continued for such a long period as to cause degradation of the fibers. As noted above, the process of the invention is rapid so that effective results are obtained in a matter of minutes, for example 2 to 6 minutes, and in no case is the time of reaction more than 10 minutes.

Following the treatment with the steam-ozone mixture, the treated material may be acidified, for example, by dipping it into a bath of dilute hydrochloric or sulphuric acid. Typically, this step is accomplished by immersing the material in 0.1 N HCl for 1 to 3 minutes. This acidification acts to restore softness of hand to the treated material and to restore its original resistance to abrasion. The acidification procedure is, however, optional and need not be applied if subsequent dyeing is planned as the acid or salt used in the dyebath accomplishes the same purpose.

The process of the invention is applicable to animal fibrous materials such as wool and mohair and these materials may be in any of various physical forms, e.g. bulk fibers, slivers, roving, top, yarns, felts, woven textiles, knitted textiles, or even garments or garment parts.

The invention is further demonstrated by the following illustrative examples:

*Example I*

Steam at 100° C. was mixed with a stream of ozone gas (50 mg. ozone per liter) issuing from an ozone generator. In the different runs the proportions of the two initial streams (steam and ozone) were varied to provide different ozone concentrations in the composite stream.

In each run, steam-ozone mixture was introduced at a flow rate of about 0.1 cu. ft./min. into a chamber wherein it was forced through a sample of wool cloth. In each case the time of treatment was 3 minutes.

Following the treatment, the treated wool samples were tested for shrinkage by the following test:

*Standard shrinkage test.*—The tests for shrinkage referred to below were conducted in the following way: The wool samples were milled at 1700 r.p.m. for 2 minutes at 40-42° C. in an Accelerotor with 0.5% sodium oleate solution, using a liquor-to-wool ratio of 50 to 1. After this washing operation the samples were measured to determine their area and the shrinkage was calculated from the original area. With this washing method, samples of control (untreated) wool gave an area shrinkage of 42%. The Accelerotor is described in the American Dyestuff Reporter, vol. 45, p. 685, Sept. 10, 1956.

15 A sample of mohair top was treated as described above in Example I, run 4, i.e. temperature 75° C., time 3 minutes, ozone concentration 31.4 mg./liter. (The expression "top" is used in the trade to designate the fiber product which has been produced by scouring the raw fleece, applying carding, combing and doubling to produce a thick strand, about 1½" in diameter, of fibers in more or less parallel arrangement, i.e. with no twist. Top is thus the refined material which is eventually treated by roving and spinning to make yarns.)

20 25 In order to test the cohesive forces between the individual fibers in the treated top, the material was placed in a test instrument where it was clamped between jaws spaced 8" apart and subjected to elongation while measuring the tensile force. Because of the wide spacing of the jaws, the results do not relate to tensile strength of individual fibers but rather to the degree to which the fibers hold to another by cohesive forces. It was found that the treated top broke at 6.5 lbs. whereas untreated top broke at 1.5 lbs.

30 35 Having thus described the invention, what is claimed is:

1. A process for improving the properties of animal fibers selected from the group consisting of wool and mohair, in particular to improve their shrinkage resistance, enhance their rate of dye absorption, and increase the cohesive forces between individual fibers which comprises mixing a stream of steam with a stream of ozone to provide a composite steam-ozone stream having a temperature about from 60 to 95° C. and an ozone concentration about from 10 to 50 mg./liter, blowing said composite stream through a mass of animal fibers for a period in the range about from 1 to 10 minutes, sufficient to attain said improvements but insufficient to cause degradation of the fibers.

45 50 2. The process of claim 1 wherein the animal fibers are wool.

55 55 3. The process of claim 1 wherein the animal fibers are mohair.

*References Cited in the file of this patent*

**UNITED STATES PATENTS**

|           |                  |                |
|-----------|------------------|----------------|
| 1,628,484 | Wilkinson        | May 10, 1927   |
| 1,825,178 | Coghill          | Sept. 29, 1931 |
| 3,086,534 | De Gorter et al. | Apr. 23, 1963  |

**FOREIGN PATENTS**

|         |        |               |
|---------|--------|---------------|
| 593,933 | France | Sept. 2, 1925 |
|---------|--------|---------------|